

# UNITED STATES PATENT OFFICE.

WALTER R. WADE, OF BROOKLYN, NEW YORK.

## PROCESS OF DEGUMMING AND PREPARING FIBERS.

SPECIFICATION forming part of Letters Patent No. 449,454, dated March 31, 1891.

Application filed May 22, 1890. Serial No. 352,781. (No specimens.)

*To all whom it may concern:*

Be it known that I, WALTER R. WADE, of Brooklyn, in the county of Kings and State of New York, have invented a new and useful Improvement in Processes of Degumming and Preparing Fibers, of which the following is a specification.

My invention consists of a new process of degumming and preparing fibers derived from ramie, hemp, flax, &c., so as to fit them for the use of manufacturers in the production of the finest textile fabrics, as herein-after fully described and claimed.

In practicing my invention I take the fiber from any of these plants as it is removed by the decorticator, of which there are numerous varieties in the market, all more or less effective in decorticating the plants—that is, peeling the bark containing the fiber from the same and separating it from the woody stems—in which condition the different fibers, notably ramie, can be had in the various markets of the world, although the fibers of flax and hemp are often still freed from their adherent woody stems by a different process. Any of the above fibers I boil in an aqueous alkaline solution of potash or soda and saponine until the gum is dissolved and the strands separated into the smaller fibers of which they are composed. The proportions of potash or soda and saponine may be varied within considerable limits for any one of the above-named fibers, and with different samples of the same fiber should be varied, to some extent, as the quantity and quality of the gum by which the fibers are agglutinated differ in these different plants and in the different lots of the same plant.

A man skilled in the art of treating fibers will through the exercise of his acquired skill vary the proportions of the alkali and saponine by observing its action upon each different lot which he is treating or preparing. To give ramie as an illustration, as without its undergoing a previous chemical preparation the fiber is unsuited for the manufacture of the finer textile fabrics, it may be prepared as follows: Take the decorticated fiber, as above described, boil it at a pressure of from thirty-five to fifty pounds from four to five hours in an aqueous solution of caustic soda

of the strength of from one and one-half to two and one-half degrees of Baumé's areometer, (temperature 60° Fahrenheit,) to which has been added from half an ounce to one ounce of crude saponine to every hundred gallons of the alkaline solution, the strength of the solution within the above limits varying according to the purity of the articles used, the amount of pressure employed, and the maturity reached by the plants from which the fibers have been obtained, which latter is easily recognized by the experienced eye. As soon as this process has dissolved the gum from the fiber, which is evident from the separation of the fine fibers which compose the largest fiber-strands in their raw state, I cleanse the fiber from the solution and the gum by washing and pressing. A very good way is to remove the fiber from the solution, wring it or press it until comparatively dry, then wash it, and finally wring or press out the water. I now immerse the fiber in a bath of acidulated water, making the bath of such strength as not to permit the acid to injure the fiber. Sulphuric acid will do, taking about one pound of the ordinary commercial sulphuric acid to one hundred gallons of water. After remaining in this bath, usually only a few minutes, I take the fiber out of the bath and bleach it by application of ordinary known bleaching agents. When the fiber is sufficiently bleached, I rinse it in water to remove the bleaching agent, and then boil it in a weak alkaline bath containing soft soap or other equivalent saponaceous material until the fiber is sufficiently softened to be fit for use, and then allow it to cool gradually, after which I wash or rinse it, when it is ready to be made into threads or yarn by the manufacturers and to be manufactured into any known way.

What I claim as my invention, and desire to secure by Letters Patent, is—

1. The herein-described process of degumming and preparing fibers, consisting in boiling them in an alkaline solution containing saponine.
2. The herein-described process of degumming and preparing raw fibers, consisting in boiling the raw fiber in an alkaline solution of potash or soda and saponine and subjecting

the fiber thus boiled to the action of a bath of acidulated water.

3. The herein-described process of degumming and preparing raw fibers, consisting in dissolving the gum by the action of an alkaline solution of potash or soda containing saponine, washing out the solution and the dissolved gum, subjecting the washed fiber to a

bath of acidulated water, and boiling the fiber in a slightly-alkaline bath containing soft soap or other saponaceous material.

WALTER R. WADE.

Witnesses:

HENRY B. LOTHROP,  
GERTRUDE H. ANDERSON.